

## [54] METHOD OF PAVEMENT REPAIR

[76] Inventor: Charles H. McDonald, 3130 W. Pierce St., Phoenix, Ariz. 85009  
 [21] Appl. No.: 784,615  
 [22] Filed: Apr. 4, 1977

|           |         |                 |          |
|-----------|---------|-----------------|----------|
| 3,253,521 | 5/1966  | Endres .....    | 404/90 X |
| 3,272,098 | 9/1966  | Buchholtz ..... | 404/32   |
| 3,400,644 | 9/1968  | Baskin .....    | 404/35X  |
| 3,568,579 | 3/1971  | Hoad .....      | 404/35   |
| 3,891,585 | 6/1975  | McDonald .....  | 404/32 X |
| 3,915,581 | 10/1975 | Copp .....      | 404/32   |
| 3,930,100 | 12/1975 | McDonald .....  | 428/323  |

## Related U.S. Application Data

[63] Continuation of Ser. No. 683,381, May 5, 1976, which is a continuation-in-part of Ser. No. 585,836, Jun. 11, 1975, which is a continuation of Ser. No. 376,915, Jul. 5, 1973, which is a continuation-in-part of Ser. No. 589,190, Oct. 21, 1976.  
 [51] Int. Cl.<sup>2</sup> ..... E01C 7/35  
 [52] U.S. Cl. ..... 404/75  
 [58] Field of Search ..... 404/72, 75, 77, 82, 404/76, 95, 17; 260/33.6 A; 106/DIG. 7, 273 R

## [56] References Cited

## U.S. PATENT DOCUMENTS

|           |        |                 |        |
|-----------|--------|-----------------|--------|
| 1,661,828 | 3/1928 | Hopkinson ..... | 264/31 |
| 1,823,682 | 9/1931 | Finley .....    | 404/72 |
| 2,977,864 | 4/1961 | Pullar .....    | 404/32 |

Primary Examiner—Nile C. Byers

Attorney, Agent, or Firm—William G. Lane

## [57]

## ABSTRACT

A method of repairing pavements employing an elastomeric pavement repair composition comprised of paving grade asphalt and rubber. The asphalt is heated to an elevated temperature and the rubber is combined therewith. The resulting composition is mixed to form a hot jellied composition which is applied to cracked or distressed pavements to repair the same. The resulting composition can also be formed into a ready made elastomeric cold patch which is applied to cracked pavement surfaces after tacking of the surface.

31 Claims, 7 Drawing Figures





FIG. 3.



FIG. 5.



FIG. 6.



FIG. 7.

## METHOD OF PAVEMENT REPAIR

This is a continuation, of application Ser. No. 683,381, filed May 5, 1976, a continuation-in-part application of my pending U.S. Pat. Application Ser. No. 5 585,836, filed June 11, 1975 which is a continuation of my U.S. Pat. Application Ser. No. 376,915, filed July 5, 1973 which in turn is a continuation-in-part of my U.S. Pat. Application Ser. No. 589,190, filed Oct. 21, 1966 on An Improvement In The Material And Its Application 10 For The Repair of Asphalt And Asphalt-Type Pavement Fractures, which are incorporated by references herein.

## BACKGROUND OF THE INVENTION

The increasing volume of traffic, and particularly heavy traffic, has created a severe problem on many roads and streets in this country. This problem has resulted from elastic type failures in pavements which cause a "chicken-wire," or "alligator" cracking pattern in the pavement surface. This cracking is caused by fatigue of the pavement surface from repeated deflection. Conventional repairs by asphalt overlays are usually effective for a short period only and many other more drastic major repairs such as replacing the pavement surface or the pavement surface and its foundation, are too expensive and often as ineffective as asphalt overlays.

The so-called "flexible-type pavement" is actually not a particularly flexible structure. There are occasions when flexible-type pavements could be classified as very brittle, particularly in cold weather or when the pavement surface has suffered a long period of embrittlement from oxidation and age. The cracking caused by this lack of flexibility has created a tremendous problem, when considered on a nation wide scale. Traveling over the streets and highways of this country, one can seldom go more than a few miles without finding distressed pavement which is basically caused by repeated flexing by the surface of the pavement under the traffic 40 loads.

This type of failure has been variously defined as flexure cracking, elastic-type failure, and fatigue failure. It is characterized by multiple cracking of the "chicken-wire," or "alligator" type pattern without plastic deformation of the pavement surface. The cracking is due to fatigue of the bituminous pavement mixture from repeated deflection of the pavement surface under vehicle load and subsequent recovery of the pavement surface. This deflection and recovery is caused by elasticity of 45 some member of the substructure or foundation of the pavement surface. Fatigue failure is the most prevalent of the three most common types of failure occurring in flexible-type pavements. The other types of failure are:

1. The plastic type of failure, which is manifested by cracking in the pavement surface of the same character as found in elastic-type of failure, but is also accompanied by plastic deformation of the pavement surface. The surface is depressed under the loaded area and usually slightly raised at one or both sides of the loaded area. This type of failure is usually caused by an inadequate thickness of base material and is no longer a serious problem on highways or streets built under modern design criteria; and
2. The surface-type failure, which is characterized by attrition, or stripping and emulsification of the asphalt in a surface of the pavement. There is ravel-

ing and loss of material in the surface but no significant amount of cracking in the surface. Although this type of failure is very common, it is not as serious as fatigue-failure because it can be corrected by the application of a seal coat.

Fatigue cracking resulting from elastic-type failure is entirely different from the above two types of failure, and solutions to fatigue cracking have not only been difficult and expensive, but in many cases quite uncertain in their result because there is resilience in some member of the substructure. This resilience must be counteracted by either making the substructure or the surface so rigid that it cannot bend, or by making the surface so flexible that it will take the bending. Part of the difficulty in solving this problem lies in the fact that the deflections required to produce elastic-type failure are so small that almost complete elimination of the resilience in the substructure is required. Repeated deflections of a very small order are sufficient to produce this type of failure. Various authorities have given figures for a critical deflection which range from 0.010 to 0.050 inches with a certain probability that the critical deflection would vary considerably for pavements of different thicknesses, composition, asphalt grade, asphalt content, asphalt quality, prevailing temperatures, and a radius of the deflection curve (see McDonald, C. H.; The Elastic Type of Pavement Failure and Some of Its Causes; 38th annual Conf. of WASHO; (2) Hveem, F. N.; Pavement Deflections and Fatigue Failures; HRB BULL. 114 pp. 43-79, 1955; (3) McDonald, Charles H.; The Flexural Failure of Sand-Asphalt Mixes as Related to Resilient Subgrades, Highway Materials Conf., Denver, CO, 1959.).

Complicating the solution to the problem of repairing fatigue cracking from elastic-type failure is the fact that the source of such a small magnitude of elasticity may be difficult to determine. The elasticity may be either in the subgrade, subbase, or base course. An increase in the normal moisture content of even a good subgrade, caused by frost action for instance, may cause the subgrade to become "quickie" resulting in a condition where vehicle load is born by hydrostatic pore pressure. Although such a condition does not ordinarily last for a long time, there is almost no reasonable thickness of overlying material or pavement that will prevent the deflection caused by the vehicle load on the pavement surface. The pavement surface of a four foot fill over a quickie soil has been observed to visibly deflect under vehicle load. This condition also develops in densely graded base courses through frost action.

Certain materials present in soils, such as mica, have elasticity within themselves, and the economic necessity of using local materials may require that these materials be incorporated in the structure. Such materials are often the only ones available in the particular area that can be used without incurring excessive costs for preparation and construction of the substructure. Perhaps the most common cause of substructure elasticity is entrapment of minute quantities of air in fine-grained subgrade soil. Any soil which is capable of moderate capillary pressure can entrap air under certain moisture conditions by holding it in pores which are sealed on all sides by capillary moisture. Capillary pressure is sufficient to prevent the air from being expelled under traffic loading. If enough of these entrapped air cells are involved in a substructure, the structure has a pneumatic character. In extreme cases such soils have an almost rubber-like elasticity when pressed between the fingers. The

moisture content need only be slightly above optimum to entrap air. This type of soil is surprisingly prevalent throughout the United States. In my opinion, the increasing use of cement-treated bases is, whether recognized or not, an attempt to overcome this problem of substructure elasticity by stiffening the substructure with cement. The so-called "up-side-down" method of construction in which the subbase is cement-treated, rather than the base, is quite obviously an attempt to stiffen the substructure against resilience from an underlying member. This is practiced rather commonly in New Mexico and Arizona (see Johnson, Charles W.; "Comparative Studies of Various Combinations of Treated and Untreated Bases and Subbases for Flexible Pavements", ARB BULL. 289, p pp. 44-56, 1961; and Arizona Highway Department, Special Provisions, Interstate Projects on I-10-4, "Tucson to Picacho Peak".)

The use of rigid portland cement concrete pavements has also been quite effective; however, the cost is generally prohibitive for indiscriminate use. Again, the obvious motive in using rigid concrete pavements is to make the pavement structure so rigid that it will not be affected by resilience of the substructure.

An attack against this type of failure, elastic-type failure, has also been mounted from the other standpoint of attempting to make the bituminous mixture more flexible (see McDonald, Charles H.; The Need for Greater Flexibility in the Surface of Flexible Type Pavements, Conf. on Soils Eng., Univ. of Ariz. Tucson, 1954). This has been done by the use of open-graded plant mixes employing very heavy asphalt films on each aggregate particle of the pavement mixture. These mixes have large void spaces so that the high asphalt content, in relation to surface area, will not cause distress. This type of pavement design has helped to ameliorate the situation, but it has not been a cure all.

Similarly, small percentages of rubber incorporated in mixes have also been used. These small percentages of rubber have undoubtedly been beneficial, although information on the degree of success obtained with these mixes for this purpose appears to be somewhat limited. It is my opinion, that the cost of these materials has prevented the use of rubber in the amounts necessary to give the pavement true elasticity. I recognized that an entirely new approach was needed to repair pavements subject to elastic-type failure and that the approach I developed and invented, which is described below, is completely different in its use of rubber from anything which I have read. My approach embodies the use of a relatively high percentage of rubber, combined with asphalt, in a relatively thin application to the pavement surface. The purpose is to keep the overall cost in balance but still obtain maximum elasticity of the patching material. This approach is unique and, to this date has been completely successful in some extremely difficult situations.

Asphalt-rubber compositions are described and claimed in many patents; however, none of these patents disclose the unique elastomeric material that I have prepared from rubber and asphalt. Preparations of asphalt containing rubber have been prepared in the past by workers in the art. For example, the Wilkinson U.S. Pat. No. 108,666 discloses a roofing compound composed of ground anthracite coal, ground gypsum, ground tan-bark, India rubber dissolved and prepared coal tar and/or commercial pitch. In the Tickstone U.S. Pat. No. 1,590,644 a hard composition containing rub-

ber and bitumen is disclosed which is useful as a substitute for porcelain, earthware, ebonite, vulcanite and the like is disclosed. This composition contains principally slate powder and lesser amounts of ground rubber and optionally bitumen and/or coloring matter. The Sadler U.S. Pat. No. 1,758,913 discloses a rubberized-asphalt mixture which is useful as a road covering. The mixture is prepared by adding aggregate to a pug mill; adding liquefier or asphalt-solvent to saturate the entire aggregate; adding rubber to the saturated aggregate so the finished mixture contains only one-half of one percent rubber based on the weight of the total asphalt added; adding asphalt or other bituminous material to the mixture at a temperature of 250° F. or higher. The Grant U.S. Pat. No. 2,040,256 discloses a rubberized-asphalt composition for sealing pipe joints and the like. The composition is prepared by melting asphalt at a temperature not in excess of 180° C. (375° F.). Ground tacky rubber is added to the molten asphalt. The resulting mixture is raised to a temperature of 245° C. (475° F.) for a period of not less than 10 minutes. The temperature is maintained while the mixture is stirred until no lumps of rubber are detectable in the mixture. The resulting composition consists of 0.5 to 15% rubber and 99.5 to 85% asphalt. The ductility of the composition is slightly less than that of the asphalt and its penetration is not more than 2% less than that of the asphalt. The Rhodes et al. Pat. No. 1,884,240 discloses a rubberized-tar product prepared by heating and stirring rubber, water-gas tar and coal tar and/or pitch until a homogeneous mass is obtained. Sulfur is added to the mixture and thoroughly mixed therein. The Taylor U.S. Pat. No. 2,686,169 discloses a method of incorporating rubber latex into hot bitumen, the resulting composition contains 2 to 6% rubber. The Endres et al U.S. Pat. No. 2,700,655 discloses a powdered rubber-containing composition for incorporation in the asphalt. The powdered composition contains from 10 to 50% rubber and from about 90 to 50% filler. Dasher U.S. Pat. No. 2,853,742 discloses a method of producing powdered rubber from scrap vulcanized rubber material which can be employed for mixing with asphalt for the production of bituminous concrete paving mixtures as well as in the production of various types of asphalt coatings and similar compositions in which it is desired that a portion of the rubber be present in the coating. The rubber is prepared in a Banbury machine. The Endres et al U.S. Pat. No. 3,127,367 discloses a method and apparatus for adding latex to hot asphalt to obtain a composition containing between 1 and 2% rubber. The Endres et al U.S. Pat. No. 3,202,623 discloses a dry, powdered rubberized composition for incorporating into asphalt. The composition is prepared by combining a water suspension of hard bitumen with rubber latex and then co-precipitating the mixture by means of a coagulant to yield a product containing 5 to 40% by weight rubber. The Peaker et al U.S. Pat. No. 3,242,114 discloses a method of dispersing a rubber-resin composition into asphalt. The resulting composition contains from 1 to 20 parts of rubber per hundred parts of asphalt. The Endres U.S. Pat. No. 3,253,251 discloses paving blocks composed of rubberized bitumen cement and rubber aggregate. This invention can be visualized as blocks of aggregate rubber particles bound by rubberized-asphalt cement. The rubberized bitumen cement contains a very small percentage of rubber.

A commercial product, Ramflex, a powdered rubber specially devulcanized in less than 5 minutes for use in

combination with asphalt and aggregate, for asphaltic-type pavement is produced by the U.S. Rubber Reclaiming Company, Inc. RAMFLEX rubber is mixed in a pug mill with asphalt and aggregate. Five to ten percent of RAMFLEX rubber is used for each part of asphalt employed in the total mixture. The total mixture is prepared by adding hot stone or sand and filler to a pug mill in the usual manner; then RAMFLEX rubber is added to the pug mill and mixed 10 to 20 seconds; finally the asphalt is mixed therein for an additional 30 seconds. The material is then ready for application.

The above patents show that rubberized-asphalt compositions are old in the art. However, not one of the previous workers in the field made the startling discovery that when certain portions of rubber and asphalt are heated and mixed together a jellied composition is formed which makes an excellent elastomeric paving repair composition.

#### SUMMARY OF THE INVENTION

The present invention is directed to a method of repairing pavements, such as roads, run ways, walk ways, and roofs, which are subject to cracking, especially fatigue-type cracking characterized by an alligator cracking pattern. The method comprises preparing a hot asphalt-rubber elastomeric material and applying it to the area to be repaired. The area to be repaired is first cleaned of all loose debris and then the hot elastomeric material is applied thereto. Before application of the hot elastomeric material, the pavement area to be repaired can be tacked with a binder such as cut-back asphalt, hot tar, and the like.

The present method is especially useful for the repair of relatively large areas of cracked pavement. The asphalt and rubber are heated and mixed at the site and then spread with conventional equipment to a depth of less than one-fourth inch, although other thicknesses can be applied. Aggregate, such as crushed rock or gravel, is then spread on the surface of the asphalt-rubber elastomeric mixture as a dressing, for the purpose of taking the abrasive wear of traffic. When the asphalt-rubber mixture is applied hot, a tack coat can often be omitted. Under the present method of repair, the surface, the base and sub-grade of the pavement do not have to be dug up and replaced with new materials as would be necessary for permanent repair of the pavements by existing methods.

The present invention is directed to a method of repairing pavements, such as roads, run ways, walk ways, and roofs, which are subject to cracking, especially fatigue-type cracking characterized by an alligator cracking pattern. The method comprises applying a prefabricated cold patch to the area to be repaired. The area to be repaired is first cleaned of all debris. Before application of the elastomeric patch, the pavement area to be repaired is tacked with a binder such as cut-back asphalt, hot tar, and the like. The cold patch is applied to the tacked area.

The present method is especially useful for the repair of relatively small areas of cracked pavement. Under the present method of repair, the surface, the base and subgrade of the pavement do not have to be dug up and replaced with new materials as would be necessary for permanent repair of the pavements by existing methods.

Repair of pavements employing the elastomeric cold patch is analogous to binding wounds with a "Band-Aid" surgical dressing and is an original and unique application of the repair patch principle. The prefabricated patch employed in the present method will be synonymously referred to herein as the prefabricated elastomeric cold patch, the elastomeric cold patch, the elastomeric patch, the cold patch and the patch.

Repairs made with the present patching material are more permanent than those made with existing materials because they are completely elastic and do not crack under repeated deflections as do conventional patching materials. A high percentage of the maintenance costs of repairing asphalt surfaces arises from the fact that repeated repairs of the same location, caused by movement of the sub-structure, are required when fatigue-type cracking of pavement is involved.

The elastomeric material of the present invention is a formulation of paving grade asphalt with penetration ranges of 10 through 300 and commercially-processed reclaimed rubber or unprocessed rubber buffings and aggregate (crushed rock, gravel, or stone). The asphalt and rubber are combined in proportions and at temperatures to form a gel which, when cooled, results in a tough, elastic mass. The mineral aggregate is added either to the hot mixture of asphalt and rubber, or subsequently after application.

The use of asphalt containing rubber in such high percentages and temperatures as to cause gelling in the formation of a completely elastic mixture when heated, fortified with crushed rock for wearability, is unique in its formulation and its application for pavement repairs. Previously known uses of combinations of asphalt, rubber and aggregate in surface applications for repair of asphalt roadways have depended upon the aggregate component for the body of the mixture. Approximately 95% of the prior art mixture would be aggregate and the remainder would be asphalt containing about 5% rubber, that is rubber would constitute 0.25% of the total mixture. The resultant conventional repair mixture is a stiff and relatively non-elastic mass when cooled that can only absorb limited pavement movement without cracking.

The unique concept in the elastomeric material of the present invention and its application lies in the fact that the asphalt-rubber component is depended upon for the body of the mixture in contrast to aggregate as in the prior art mixtures. In the present application, the final patch is comprised of approximately 10 to about 50% of the elastomeric material and about 50% to about 90% of aggregate although smaller and larger amounts of aggregate can be used. By making the rubber content of the elastomeric material high enough (approximately 25 to 33%) a solid is formed when the rubber and asphalt are heated to a gel and are allowed to cool which is completely elastic and will move with the underlying surface without cracking. In the present application, the aggregate component only takes the abrasive wear of traffic and does not constitute the working body of the mixture. In the present application, the aggregate may be used as a dressing only instead of being mixed integrally.

I have found that a rubber-asphalt material could be made to have the consistency of a thick slurry or gel when hot which forms a tough elastic mass when cooled. I have found that the best consistency for our purpose could be obtained by heating paving grade asphalt to from about 350° and about 500° F. and then stirring into it rubber, such as partially devulcanized reclaimed rubber (a commercial product), in the proportion of about two to three parts of asphalt to about one part of rubber. The laboratory tests showed that the

consistency of the final product depended not only on the rubber content, but also on degree of solution or jelling and surface interaction of the rubber. The higher the temperature of the mixture, the greater the degree of solution and surface interaction of the rubber and the asphalt and the more nearly the end product resembled the properties of rubber rather than asphalt. In other words, when the material is mixed briefly at a temperature of 350° F. it is quite fluid and has a consistency of a thin slurry. This would be very convenient for placing; on the other hand, it would be more temperature susceptible so that it would tend to bleed more readily in the summer, be more brittle in cold weather, and would have less elasticity than a thicker product. A similar situation occurs when the rubber content of the material is reduced. In other words, the material can be made at any consistency desired, but it must be remembered that in doing so the properties of the final product will be changed. The thinner the hot product, the more nearly its properties will resemble those of asphalt and the thicker the hot product given the same proportions of rubber and asphalt, the more the end product will resemble rubber.

The elastomeric composition has been prepared from a variety of rubbers, such as ordinary reclaimed rubber obtained from a local vulcanizing shop. The reclaimed rubber was a finely granulated product obtained from the buffing of tires for retreading. This material can be mixed in the proportion of about 2 to about 3 parts of paving grade asphalt to one part of reclaimed rubber. Ground whole tire rubber, asphalt soluble rubber, unprocessed rubber tire buffings and salvaged tire rubber can also be used in the elastomeric material.

The claimed elastomeric material consists essentially of asphalt and rubber of certain proportions which have been heated together within a specified temperature range to form a jellied composition. The claimed material consists essentially of paving grade asphalt and rubber in the ratio of about 2-3 to about 1 by weight respectively. The asphalt is heated to a temperature between about 350° and about 500° F. and the rubber is mixed therein to form a reaction product, the jellied composition. This elastomeric material has several exceptional and unexpected properties. For example, it does not reflect underlying fatigue cracks after application on the cracked distressed pavement. As shown above, the conventional pavement repair materials such as hot mix, sand-asphalt and slurry seal cannot be successfully employed to repair cracked-distressed pavements because cracks reflect through the repair material. Surprisingly, the claimed elastomeric material can be used to successfully repair cracked-distressed pavement by merely covering the surface of the pavement with a thin layer, e.g. about one-fourth inch thick, of the hot elastomeric material. In addition, the elastomeric material has excellent and unexpected weatherability and wearability on pavement. For example, several cracked-distressed pavements repaired with the elastomeric material have been subject to severe inundation without any detrimental effects on the claimed material (see the examples). The claimed elastomeric material has shown exceptional wearability under severe traffic conditions as shown in the examples. As of 1973, seven years after the preparation, two of the panels of Example 1 are still in service. The other panels, as described in the examples, were destroyed when the streets were rebuilt. Because of its repair, weatherability and wearability characteristics, the claimed invention has seen

widespread commercial use, such as on highways, mountain roads, desert roads, airport, runways, and city streets over the last several years.

The novel elastomeric composition of the present invention on a weight basis is not as inexpensive as conventional repair materials. However, the cost of the material is not out of line with heavier overlays which are commonly used and generally unsuccessful in combating the problem of fatigue cracking, or with slurry seals also commonly used and generally unsuccessful in preventing reflection cracking. In maintenance repair work, the cost of the material is relatively a minor item. The big cost item in maintenance repair work is the labor involved. A product that will eliminate repeated repairs to the same distressed pavement area has a tremendous economic advantage over the conventional repair materials. Moreover, the present composition is applied to the pavement in relatively thin layers between one-twentieth and one-half inch in thickness. Since the material can be laid in relatively thin layers the economics of the present product are not out-of-line when compared with conventional materials.

The elastomeric patch material of the present invention will flow into the chicken-wire or alligator pattern cracks and bond the fractured pavement together with an elastic bond to prevent further surface cracking and penetration of moisture. Other materials used for this purpose, such as asphalts, or asphalts with little rubber content, are primarily plastic with little or no elasticity to take or recover from repeated deformation, particularly in cold weather when they become very brittle. The elastomeric material of the present invention is unique in that it retains some flexibility under all weather conditions.

#### DESCRIPTION OF THE DRAWINGS

FIG. 1 illustrates a cut-away perspective view of an alligator crack pavement surface repaired by the present method;

FIG. 2 illustrates a cross-sectional view of a repaired alligator crack pavement taken along lines 2-2 of FIG. 1;

FIG. 3 illustrates a cross-sectional view of a road prepared by the present method;

FIG. 4 is a cross-sectional view of one embodiment of the cold patch used in the method of the present invention;

FIG. 5 is a cross-sectional view of one embodiment of a road constructed by the present method;

FIG. 6 is a cross-sectional view of another embodiment of a road constructed by the present method; and

FIG. 7 is a cross-sectional view of a pavement structure prepared according to the present method.

#### DETAILED DESCRIPTION OF THE INVENTION

The elastomeric paving repair composition is prepared by heating paving grade asphalt with a penetration range of 10 through 300 to a temperature within the range of from about 300° to about 500° F. and adding particulate rubber (one-half inch to +200 mesh USS) thereto. The resulting mixture is thoroughly mixed until the composition gels or becomes jellied. No additional heating is required once the rubber is added to the asphalt. About one part rubber is added to each two to three parts asphalt. I have used 85-100 penetration grade asphalt in my test work for convenience although other penetration grades of paving asphalt such as

120-150 grade are equally suitable and are generally used for practice of the invention.

The elastomeric cold patch employed in the present method is prepared from the elastomeric paving repair composition. The hot elastomeric material is applied to sheets of paper, cardboard, fabric or plastic to form a layer of hot material on the sheet. Preferably the patch is formed in a form to give a patch of relatively uniform depth. Normally between  $\frac{1}{2}$  and about 1 gallon of the hot elastomeric material are applied per each square yard of sheet. However, lesser amounts, such as  $\frac{1}{4}$  gallon per square yard or greater amounts such as  $2\frac{1}{2}$  gallons per square yard can also be applied. When the hot composition cools, the layer of hot elastomeric material normally is from about 0.2 to about 0.25 inches in thickness. However, thinner layers such as paper-thin layers or thicker layers, such as layers an inch thick, can also be formed and used. After application of the hot elastomeric material and before it cools, and sets up, the layer is dressed with an aggregate cover that is preferably tamped or rolled into the elastomeric material. Between about 20 and about 50 pounds of conventional mineral aggregate or about 5 to about 20 pounds of light weight aggregate are used for each square yard of the composition layer, preferably between about 25 to 40 pounds of conventional mineral aggregate per square yard. Nominally sized aggregate of  $\frac{1}{4}$  or  $\frac{3}{8}$  inch is normally used; however, smaller sized aggregate such as sand or larger aggregate sizes can also be employed. The resulting product is then allowed to cool to form an elastomeric cold patch. The patch can be cut, if desired, into various sizes and shapes.

Alternatively, after the hot elastomeric material has been prepared that is the hot jellied composition, aggregate, preferably preheated to a temperature between about 300 and about 500° F., can be added to the hot composition before it is applied to the paper or cardboard sheet. In this method of preparation, we have employed about equal weights of aggregate with equal weight of the hot composition. However, the end product will preferably have between about 20 and about 50 pounds of aggregate per square yard of the cold patch, preferably between about 25 and 40 pounds of aggregate per square yard of cold patch.

The cold patch of the present invention also can be prepared without a sheet backing. The hot elastomeric material is applied to a nonadhesive surface to which the hot elastomeric material will not adhere such as a plastic or Teflon resin coated surface. The aggregate can be added to the composition before it is applied to the surface or it can be applied afterwards and tamped and rolled therein. The composition is applied at such a rate that the thickness of the resulting cold patch is normally between about 0.2 and about 0.25 inches in thickness. However, the thickness of the elastomeric cold patch layer can be thinner, such as about 0.1 inch in thickness, or thicker, such as about 0.5 inch in thickness, as described above. The cold patch after cooling should be treated with a material that will prevent sticking of the cold patch to other surfaces. Lime has been found to be an ideal material for this application. However, other adhesive breaking types of materials known to the art to prevent sticking and tacking can also be used. An adhesive breaker when applied to the surface of the patches, inhibits the patches from sticking together, especially when the patches are stored in stacks.

Hydrocarbon rubbers are used in the present inventions. By the term "hydrocarbon rubber" is meant non-

oil resistant asphalt-soluble rubbers. Non-oil resistant asphalt-soluble rubbers are those rubbers that are partially soluble to the extent from about 2 to about 12% by weight in asphalt and are attacked by, react with, or are affected by oils, such as lubricating oils, hydraulic oils and the like. Suitable rubbers that can be employed include unvulcanized, vulcanized or reclaimed rubbers including natural rubber, (NR, polyisoprene polymer), isoprene rubber (IR, polyisoprene polymer), butadiene rubber (BR, polybutadiene polymer), butadiene-styrene rubber (SBR, butadiene-styrene copolymer), butyl rubber (IIR, the isobutylene isoprene polymer) and ethylene propylene rubber (EPM and EPDM, ethylene propylene copolymers and terpolymers) which are unvulcanized, vulcanized or reclaimed.

The reclaimed rubber can be devulcanized or partially devulcanized and can be prepared from vulcanized or unvulcanized rubber by the digester process, Heater or Pan process, high pressure steam process, Lancaster-Banbury process, reclamation or other conventional reclaiming processes (Maurice Morton, Introduction to Rubber Technology, Van Nostrand Reinhold Co., New York, 1959, pp. 404-435). Normally the reclaimed rubber will be prepared from old, worn tires, tire scrap, innertube scrap, retread scrap, tire peel, tire carcass, rubber buffings and other rubber scrap.

In the practice, other types of rubbers, that is, oil resistant and/or non-asphalt soluble rubbers have not been found suitable for preparing the hot elastomeric pavement repair material. For example, rubber which has not been found suitable for the composition are: nitrile (NBR, butadiene acrylonitrile copolymers), epichlorohydrin (ECO, epichlorohydrin polymer and copolymer), neoprene rubber (CR, chloroprene polymers), hypalon (CSM, chloro-sulfonated polyethylene polymers), urethane rubber (AU, EU, urethane polymers or elastomers), polysulfide or thiokol rubber (T, organic polysulfides), silicone rubber (Si, organic silicone polymers), fluoro silicone rubber (FSi, fluorinated organic silicone polymers), fluoro elastomer (FTM, fluorocarbon polymers), acrylic rubbers and polyacrylates (ACM, copolymer of acrylic ester and acrylic halide). These rubbers have been found to be unsuitable for the present invention because they do not react in the desired manner with asphalt under the described conditions to form the required jellied composition.

The following types of rubbers are preferred for use in the invention: (1) ground whole tire rubber (with and without carcass fabric residue); (2) unprocessed rubber buffings, that is rubber buffings that have not been subject to devulcanization or reclaiming processes (a by-product of tire retreading); (3) ground innertubes (natural rubbers and synthetic butyl rubbers); (4) reclaimed rubber; (5) partially devulcanized reclaimed rubber; and (6) asphalt soluble rubber. The preferred particle size for the rubber is from about 4 mesh to about +200 mesh USS. Unprocessed rubber refers to rubber that has not been chemically or thermally altered. Unprocessed rubber includes rubber that have been ground, screened, decontaminated, and treated to remove metals, cord and fabric therefrom.

Once the hot jellied composition has formed, the composition is applied directly to the pavement area to be repaired. The pavement area to be repaired is first swept clean of all debris and made thoroughly dry. Optionally, a tack coat of hot asphalt, solvent cut asphalt such as kerosene and asphalt, or an asphalt solvent, such as gasoline or kerosene can be applied to the

area to be repaired. Alternatively, if the pavement surface is asphaltic, the surface can be made adhesive and tacky by heating with a torch or the like. The hot elastomeric material is then applied to the area to be repaired to form a continuous layer averaging in thickness of from about one twentieth to about one half inch. Thicker or heavier layers can be applied. The hot elastomeric composition can be applied by spraying, mopping, screeding, squeegeeing, or shoveling the composition onto the pavement surface. As soon as possible 10 after application to the pavement, preferably immediately after application to the pavement, sand or mineral aggregate or chips are applied on top of the hot elastomeric material and rolled therein to provide a protective wear surface for the hot elastomeric composition. The aggregate is normally sized to one fourth or three 15 eighths inch but other size aggregate can be used.

The grading or sizing for mineral aggregate or chips used on street repair work can vary but I have found the following three-eighth inch nominal size chip very successful:

| Sieve Size | % Passing |
|------------|-----------|
| 1/8"       | 100       |
| 1/4"       | 70-100    |
| #8         | 0-5       |
| #200       | 0-2       |

The chips can be optionally treated with asphalt to eliminate the dust problem. The chips are coated by 30 heating them to a temperature between 250° and 325° F. and pre-coating them with a small amount of asphalt. With three eighth inch nominal size chips the application rate is about 25-40 pounds of chips per square yard of hot elastomeric material.

When repairing pavements in the airport area, we prefer to use one fourth inch nominal chips because there is less hazard that the chips will be torn loose from the elastomeric material and sucked into the jet engine where they can do severe damage. The following one 40 fourth inch nominal size chip specification have been found to be very satisfactory for airport use.

| Sieve size | % Passing |
|------------|-----------|
| 1/8"       | 100       |
| 1/4"       | 80-100    |
| #8         | 0-5       |
| #200       | 0-2       |

The hot elastomeric material can also be dressed with sand or a mixture of aggregate and sand.

Referring to FIG. 1, the alligator cracked pavement structure 10 is comprised of the top pavement layer 12, a base 14, and a sub-base 16. Pavement structures vary for different conditions; normally, however, the pavement top layer 12 consists of aggregate bound with asphalt, or concrete. The pavement layer 12 is generally 1-6 inches in thickness; however, in certain situations such as the landing area of a runway, the thickness of the layer 12 can be thicker. The base 14 normally consists of sized aggregate fill, preferably crushed aggregate. In some situations in order to give the pavement structure greater rigidity, the aggregate is cemented together with asphalt or cement. In the latter situation, there is generally a sub-base layer 16 situated below the base layer which is filled with aggregate or similar road building material. The final layer of most pavement construction is the sub-grade (not shown) which is com-

5 pacted earth which can be compacted with aggregate and/or treated with cement, asphalt or other additives.

The alligator cracks 18 generally propagate through the layer 12 however, when the base has been cemented together with asphalt or cement the cracks can also reflect through this layer. Water has a tendency to flow through the cracks and soften the underlying base, sub-base or sub-grade to eventually destroy all support for the layer 12 which then displaces downwardly.

The surface of layer 12 is first cleaned of all loose debris and dried. Optionally, the surface can be treated or tacked prior to application of the hot elastomeric repair material with a tack coat 20. The surface of layer 12 can be tacked with hot asphalt, solvent cut asphalt, such as paving grade asphalt cut with kerosene or the like, with one of the commercially available rubberized-asphalt compositions which contain up to 5% rubber, with an asphaltic solvent such as kerosene or gasoline and the like. In addition, the top surface of layer 12 can also be heat treated with a torch to make the asphalt in the pavement, assuming that pavement layer 12 is asphaltic, adhesive and tacky. However, treatment of the surface of pavement layer 12 is optional and is generally only done when the pavement surface is relatively cold, such as below 70° F. in order to insure there is a good adhesive bond between the hot elastomeric repair material and the top surface of the pavement 12.

As described above, the hot elastomeric repair material is either sprayed on, shoveled on or mopped on to the top surface of layer 12 to form a patch or panel 22. Generally, the hot elastomeric material is applied to the surface at a rate of from about  $\frac{1}{2}$  to about 1 gallon of the composition per square yard of pavement surface. However, there may be situations wherein lesser amounts, such as  $\frac{1}{4}$  gallon per square yard, or greater amounts, such as 2.5 gallons per square yard of the composition may be applied. Immediately after application, before the hot elastomeric material cools and sets up, the hot patch 22 is covered with a coating of conventional mineral aggregate 24 (see FIG. 2). Generally between about 20 and about 50 pounds of conventional mineral aggregate per square yard of the hot elastomeric patch are applied, preferably between about 25 and about 40 pounds of conventional mineral aggregate per square yard. The aggregate is tamped and rolled into the hot elastomeric material and always protrudes above the surface of the material so that there are no "bald spots" on the patch surface.

With reference to FIG. 1, when employing the elastomeric cold patch to repair cracked pavement, the surface of the pavement 12 is swept clean of all loose debris and dried. The surface is then treated and tacked prior to application of the elastomeric cold patch with a tack coat 20. In contrast to repairing a cracked pavement with the hot elastomeric material, tacking is a compulsory step when employing an elastomeric cold patch. However, the bottom surface of the cold patch can be tacked rather than surface of the pavement. After tacking, the cold patch is applied to the pavement surface and tamped or rolled preferably rolled, thereon to insure maximum adhesion between the bottom of the patch and the surface of the pavement 12 and to force out any air bubbles trapped between the underside of the patch and the pavement surface. If the patch has a release type backing, the backing is removed from the patch prior to its application to the pavement. However, if the patch has a backing that is permanent, such

as a paper backing, the backing side of the patch can face either up or down when the patch is applied to the pavement. Normally, after a period of time, vehicular traffic will wear the backing off the top surface of the patch when it faces upward.

The elastomeric cold patch is similar in structure to the elastomeric patch 22; the elastomeric patch 22 being formed on the pavement while the elastomeric cold patch is formed elsewhere by the method described above. The elastomeric cold patch is ideally suited for small cracked areas. However, a series of cold patches can be used to repair a large area, although difficulties may be encountered when sealing the adjacent side of the joints of the cold patches so that water will not seep there between. Adjacent cold patches can be permanently sealed by applying the hot elastomeric pavement repair material from which the cold patch is prepared to seal the joints.

The cold patch 25 normally has a thickness of from one twentieth to about one half inches in thickness, preferably from about 0.18 to about 0.25 inches in thickness. Each square yard of cold patch contains about 25-40 pounds of aggregate cover which has been blended, tamped or contacted into the cold patch as described herein. The top surface of the cold patch 25 is completely dressed or exposed to aggregate 24 so there are no bald spots. The aggregate protects the elastomeric composition 28 of the cold patch from abrasion and stripping by vehicular traffic.

Referring to FIG. 4, the cold patch 25 consists of a 30 backing layer 26, aggregate 24 and the elastomeric pavement repair material composition layer 28. The backing 26 can be a permanent backing or can be a release type backing. The backing is normally prepared from paper, cardboard, or plastic and if it has a release type backing, it has a coating of plastic, such as a polyvinylchloride, adjacent to the composition layer 28. The composition layer 28 is normally from about one twentieth to about one half inches in thickness, preferably from about 0.2 to about 0.025 inches in thickness. The 40 aggregate chips 24 are normally from about one fourth to about three eighth inch chips; however, smaller size chips including sand, and larger size chips can be used. The aggregate permeates the complete thickness of layer 28 and projects above the top surface of layer 28 so that no bald spots or uncovered areas are exposed.

In an alternative embodiment of the present invention, the cold patch 25 has no backing layer 26. The backing layer is generally used in order to enhance production of the cold patch and to prevent cold patches from sticking to one another when stacked or piled. However, the cold patch can be prepared without such a backing layer and can be covered with an adhesive breaker, such as talc, to prevent sticking when cold patches are piled.

Referring to FIGS. 3 and 6, a light traffic road 30 is illustrated. That is a road that does not bear a great deal of vehicular traffic, especially heavy truck traffic. The road consists of a pavement layer 32 a compact sub-grade 34, an earth sub-grade 36. The road illustrated in FIG. 3 has drainage ditches 38 on both sides of the road. The road can be quickly and rapidly prepared by grading and compacting an area to obtain sub-grade 34 over sub-grade 36. Optionally, sub-grade 34 can be compacted with gravel, sand and aggregate and/or treated with a binder, cement, asphalt, or cutback asphalt. The road can be prepared without sub-grade 34 (not shown). Optionally, the road can be constructed with an inter-

mediate layer 33 (See FIG. 5) between layer 32 and sub-grade 34 of asphalt, asphalt-concrete or concrete. At both sides of the road, drainage ditches 38 are optionally dug and formed (See FIG. 3) which are deeper than the top surface of the compacted sub-grade 34. The road can be constructed with a single drainage ditch on one side of the road (See FIG. 5) or without drainage ditches (See FIG. 6). The hot elastomeric composition of the present invention is applied over the top surface of sub-grade 34 and on bottom and back slopes of the ditches 38, if the road has drainage ditches. Optionally, the hot elastomeric composition can be applied to the outer top edges and shoulder 39, if any, of the drainage ditches 38 when composition is applied to the bottom 15 and back slopes of the ditches. Immediately after application of the hot elastomeric material and before it cools and sets up, the composition is preferably covered with aggregate at a rate of between about 20 and about 50 pounds of aggregate per square yard of the hot composition. Optionally, but preferably, the back slopes and, outer top edges and shoulder 39 of the ditches 38 are also covered with aggregate. This type of road is very easy to construct, relatively inexpensive and quite rugged when not subject to heavy vehicular traffic or frequent travel by heavy trucks. This type of road will not crack or strip because the elastomeric composition is resilient. The chief concern with this type of road is the undercutting of sub-grade 36 or sub-grade 34 by water which can destroy the foundation and support for the pavement surface 32. The undercutting can be minimized by drainage ditches and covering the ditches, their back slopes and outer top edges and shoulders with the hot elastomeric composition.

The hot elastomeric material can also be used as a waterproof and/or stress absorbing membrane interlayer for pavement application (See FIG. 7). The hot elastomeric material because of its rubber-like elastomeric properties can be applied directly over a road, pavement or other surface 40. The surface 40 of the pavement surface is cleaned of all debris and dried before application. Depending upon the weather conditions and the type of surface, the surface can be optionally tacked as described above with reference to FIG. 1. The hot elastomeric material is applied to the surface of pavement 40 either by mopping, spraying, squeegeeing or shoveling on and smoothing off to form a layer or membrane 42 of the hot elastomeric material. A thin layer having a thickness of about 0.03 to about 0.15 inch can be applied when the membrane 42 is to act as a waterproof membrane. A thicker layer, such as a thickness of about 0.1 to about 0.5 inch, preferably a thickness of about 0.1 to about 0.25 inch, is used when the layer 42 is to also act as a stress absorbing interlayer. Thereafter, the hot elastomeric material can be optionally covered with a dressing of aggregate or other suitable dressing or material in order to prevent pick up. After the elastomeric material has set and cooled, it can be covered with a layer 44 of conventional pavement surfacing materials, such as asphalt-concrete, macadam or concrete. This interlayer 42 acts as a stress absorbing membrane between the underlying foundation or base 40 and 36 and the overlying pavement layer 44. As discussed above, pavements often undergo deflection and recovery movements when subject to loads because of the elasticity of the pavement substructure or foundation. Conventional pavement materials, such as macadam, asphalt concrete or concrete do not possess sufficient flexibility to flex, without cracking, under such

deflection and recovery movement. However, the elastomeric material interlayer 42 is elastomeric and inhibits reflection of the deflection and recovery movements of the substructure or foundation 36 and 40 to the top pavement layer 44 and thus prevents cracking of the pavement layer 44.

The hot elastomeric material can also be used as a waterproof membrane for roofing application (not illustrated). The hot elastomeric material because of its rubber-like elastomeric properties can be applied directly over the roof surface and over any roof expansion joints because the elastomeric material will be able to give and take with the expansion and movements of the joints. The surface of the roof is cleaned of all debris and thoroughly dried before application. Depending upon the weather conditions and the type of surface, the surface can be optionally tacked as described above. with reference to FIG. 1. The hot elastomeric material is applied to the roof surface either by mopping, spraying, squeegeeing or shoveling on and smoothing off to form a relatively smooth thin membrane of the hot elastomeric material. Thereafter, the hot elastomeric material is covered with a dressing of aggregate or other suitable roofing dressing or material in order to prevent pick up when someone walks across the surfaced roof. Due to the ability of the elastomeric material to withstand oxidation and degradation better than asphalt alone, and its elastomeric properties, it makes a long life, tough and resistant water-proof membrane for roofing and other structures.

Although not illustrated, the elastomeric repair composition can also be applied to line earthen canals, repair cracked inner dike or dam surfaces, that is the surface exposed to the water, and it can be used to form a waterproof membrane for earthen reservoirs and the like. In all these applications, the material can be layed in a relatively thin layer such as between one twentieth and one fourth of an inch in thickness. Preferably, the elastomeric material is covered with aggregate or a thick course of earth, such as a layer of earth about 3 to about 12 inches thick, in all these applications to protect it from abrasion and pick up and other mechanical type damage.

The temperature susceptibility of the elastomeric rubber-asphalt pavement repair material is far less than with paving grade asphalt alone. This is, of course, a tremendous advantage in achieving control of reflective cracking. The elastomeric material retains some flexibility down to below freezing temperature although it does soften some under summer heat, it apparently does not soften to such a point that it is picked up by vehicular traffic. The elastomeric material will be quite soft to the touch when warm and show tracking under truck tires. However, instead of the material shoving and rolling under vehicular traffic, it rebounds and tends to resume its original location. A somewhat leathery skin develops on the surface of the elastomeric material after application and cooling which is dry and resists pickup. The elastomeric material will pick up, however, if a tacky material such as asphalt is applied to this dry surface. However, the aggregate or sand covering protects against this type of problem.

Patching by this process is comparable to that of the manufacture and placing of slurry seal. The only difference between this process of pavement repair and pavement repair with a slurry seal is that the liquid composition must be hot when applied. The hot elastomeric material after application can be smoothed out with a

rubber squeegee in the same manner that slurry seal is smoothed out when applied to a street. The similarity of the processes, ends after smoothing with the squeegee. In the case of the elastomeric rubber-asphalt pavement repair material, a cover aggregate surface is added to the composition to prevent traffic pickup. As soon as the aggregate surface has been applied and the composition allowed to cool, traffic may be allowed on the repaired surface almost immediately. In contrast, when a pavement surface is repaired with slurry seal a considerable curing time must elapse from the time of application before traffic can be permitted to use the repaired street otherwise vehicular traffic will destroy the repaired street surface.

As far as I have been able to judge there is no apparent difference in the performance of pavement repair panels made with compositions repaired with partially devulcanized reclaimed rubber and ordinary reclaimed shredded rubber obtained from a local vulcanizing shop. There is, however, a difference in the reaction of the two rubbers to asphalt. The elastomeric composition prepared from partially devulcanized reclaimed rubber seems to be a stiffer product when mixed at higher temperatures, whereas the reverse is true with elastomeric compositions prepared from conventional reclaimed rubber. The ideal temperature for asphalt, in preparation and mixing of the elastomeric composition, appears to be approximately 420° F.

A field study under my supervision was made to determine the location of the most severe test conditions that could be found for the use of the elastomeric pavement repair material. My desire was to locate pavements where the traffic was heavy, preferably with a high percentage of heavy truck traffic, and where severe elastic-type failure has already occurred. I also sought an area where poor drainage was involved and one of the test areas did have exceedingly poor drainage. Descriptions and examples of the working of the present invention are set forth in the following examples. Further information regarding the present invention can be found in my paper entitled *A NEW PATCHING MATERIAL FOR PAVEMENT FAILURES* published in the *Highway Research Record*, No. 146, pps. 1-16 of the Highway Research Board, Div. of Eng., National Research Council, National Academy of Sciences-National Academy of Engineering, Washington, D.C. (1966), which is incorporated by reference herein.

The present method can be used to repair or cover all types of pavements and surfaces. It can be used to repair pavements subject to fatigue type cracking, plastic type failure or surface-type failure. It can be used to repair pavements and surfaces that have been holed, torn or sheared.

#### EXAMPLE I

The following elastomeric pavement repair material panels were applied to a street where the traffic volume numbered 13,200 vehicles per day, a large portion of which were trucks because this street served an industrial area. The pavement surface of this street was generally covered by alligator-pattern cracking in an advanced state and the drainage was extremely poor. After a rain storm a portion of the street was frequently inundated.

An elastomeric composition was prepared from two parts of 85-100 penetration asphalt and one part of partially devulcanized reclaimed rubber. The mixture

was applied at a temperature of 420° F. at a rate of one gallon of the hot elastomeric material per square yard of pavement surface. After application, cover aggregate (mineral aggregate) was spread over the surface to prevent pick up. Traffic was turned onto the repaired surface within three quarters of an hour after application of the aggregate. This was sufficient time for curing as the material set up on cooling. The resulting layer of elastomeric material was less than one fourth inch thick. The clean-cover aggregate after spreading over the hot elastomeric material surface was tamped into the composition.

Approximately three weeks after placement of the above repair panel, the area was subject to 58 hours of steady rain and partial inundation while the street was being pounded by traffic. The test section was not affected; however, conventional sand-asphalt mixes which had been placed over adjoining areas were cracking. These same sand-asphalt panels were raveling due to partial emulsification of the asphalt. A few months later these sand-asphalt patches were almost completely destroyed, but the elastomeric pavement repair panel made of the rubber-asphalt mixture showed no reflection cracking from the underlying cracks or any other distress.

Another panel of the same composition as the above panel was applied to an area of the pavement which had been tacked with MC-250 liquid asphalt. Traffic was held off this patched area for about two hours after the application of the aggregate. This patch or repair panel was subjected to the same conditions as the above panel and held up equally as well even after being subjected to severe rains and heavy traffic, including heavy truck traffic.

An elastomeric composition was prepared from five gallons of 85-100 penetration grade asphalt and 21 lbs. of partially devulcanized reclaimed rubber (two parts of 85-100 penetration grade asphalt to one part rubber by weight). The temperature of the asphalt was 420° F. and the rubber was added thereto and mixed therein. The pavement area being repaired was initially tacked with four parts of 85-100 penetration grade asphalt diluted with five parts of kerosene. The hot elastomeric mixture was spread over the pavement area being repaired in a patch or repair panel having a thickness of one fourth to one half inches in depth. The entire panel was completely covered with aggregate and rolled with a steel roller. This panel was spread at a different rate than the foregoing panels which would average to a depth of approximately 0.18 inches thickness (1 gallon/square yard). This particular panel was spread to a depth of one fourth to one half inch and was followed with a one fourth inch cover aggregate.

The above panels until their destruction, when the street was completely rebuilt, showed no reflection cracking. The only effect that could be observed on the panels some six months after their application was a small amount of spread of the panel in the direction of traffic.

A hot elastomeric pavement composition was prepared from two parts of 85-100 penetration asphalt and one part of unprocessed shredded reclaimed rubber from a rubber tire shop. The asphalt was heated to a temperature of 440° F.; thereafter, the rubber was heated and mixed with the asphalt to form the hot elastomeric composition. The composition was applied to the pavement at the rate of one gallon of composition per square yard of surface area giving a patch having a

thickness of 0.18 inch. The pavement surface was first tacked with kerosene cut asphalt (4 parts 85-100 penetration grade asphalt and 5 parts kerosene). The hot elastomeric material after application was completely covered with one fourth inch seal coat aggregate and turned over to traffic. This panel remained in excellent condition until it was destroyed when the street was completely rebuilt. No cracking or stripping occurred up to the time of its destruction although some spreading occurred in the direction of traffic.

#### EXAMPLE II

The following elastomeric pavement repair panels or patches were situated on a street having a daily traffic volume of from 30,800 to 38,400 vehicles per day. Most of the traffic was passenger vehicle traffic. There was severe alligator-type cracking in the wheel tracks of the street but that had not spread generally over the street as the cracking had occurred in the street described in the previous example.

An elastomeric paving composition was prepared from five gallons of 85-100 penetration grade asphalt and 21 lbs. of partially devulcanized reclaimed rubber (two parts of 85-100 penetration grade asphalt to one part rubber). The temperature of the asphalt was 430° F. when the rubber was added and mixed thereto. The resulting elastomeric pavement repair material was spread over an area of 5.3 square yards to give a patch having a thickness of about one fourth to one half inch. The panel was rolled with a steel roller after placing cover aggregate. Prior to applying the hot elastomeric composition, the area repaired was tacked with a solvent cut asphalt consisting of four parts of 85-100 penetration grade asphalt and five parts of kerosene. While rolling this panel with a steel roller to set the cover aggregate, some of the hot elastomeric composition was squeezed up through the cover aggregate and the roller picked it up creating a bald spot or two. This did not appear to affect the properties of the patch, but the rolling of the hot elastomeric material when it was too hot caused an uneven penetration into the cover aggregate, resulting in a certain roughening of the surface texture. This roughness was eventually ironed out under traffic.

After a half years use, the repair panel was very soft and spreading in the direction of traffic and to the sides causing thin spots with some minor resultant reflection cracking. This panel appeared to be softer than the panels of Example I. This is probably due to a combination of an excess of tack coat and greater thickness of the rubber-asphalt material resulting in slower curing. Ideal average thickness seems to be about 0.2 inches which is obtained by spreading 1 gallon of the hot elastomeric material over a square yard of the pavement surface.

A hot elastomeric composition was prepared from fifteen gallons of 85-100 penetration grade asphalt and sixty-two pounds of partially devulcanized reclaimed rubber (two parts of asphalt to one part of rubber). The asphalt was heated to 400° F. and then the rubber was added and mixed therein to form a jellied composition. The resulting composition was applied over 20 square yards of surface area (one gallon of the hot elastomeric composition per square yard of pavement surface) and covered with a cover of aggregate. The pavement was first tacked with kerosene cut asphalt. This material was placed over a portion of a long strip of failed pavement area. The remaining portion of the same strip was re-

paired by a conventional maintenance slurry seal patch approximately a week later. The slurry seal patch showed distress after only a week of emplacement and completely failed a few months after emplacement. After five months after initial emplacement, the slurry seal patch was replaced with a hot asphaltic-concrete mix was emplaced, several slurry seal patches containing small percentages of latex were placed on adjoining areas. These patches also failed because the rubber content of the slurry seal is insufficient to give the patch the required elasticity. All the slurry seal patches had to be completely replaced approximately three months after placement. The elastomeric pavement repair patch was in good condition at this time except for small exceptionally thin spots where reflection cracking showed up to a minor degree. The one fourth inch cover aggregate used on this patch was completely covered by the elastomeric rubber-asphalt composition after a few days of traffic. In the spot where the cracking occurred, the aggregate had not been covered as there was insufficient elastomeric material to squeeze up around it. Where the normal thickness of the elastomeric composition was obtained, there was no reflection cracking.

The elastomeric pavement repair material prepared in the last paragraph above can be employed in road construction. A cut 18 feet wide is made in the earth to about a depth of 3 inches. The cut is compacted with a heavy roller and back filled for 2 inches with 1 inch to 2 inches aggregate and backed filled to the top of the cut with 1/4 inch to three eighth inch aggregate. The aggregate subgrade is covered with the hot elastomeric composition to form a layer about one fourth inch in thickness. Before the composition sets up, it is given a dressing of one fourth inch aggregate which is rolled into the layer to yield a light utility road.

The road can be optionally built with ditches on both sides of the road or a ditch on one side of the road to prevent water from eroding away the earth foundation of the road.

## EXAMPLE II

An elastomeric pavement repair patch was placed on a street which had a traffic count of 18,500 vehicles per day. Many of these vehicles are of the commercial and industrial type. This street section was in an area which had given continuous trouble for street maintenance for some time.

An elastomeric composition was prepared from two parts of 85-100 penetration grade asphalt to one part of locally obtained, unprocessed, shredded, reclaimed rubber by weight. The asphalt was heated to a temperature of 420° F. when mixed with the reclaimed rubber to form a hot jellied composition. The area to be repaired was tacked with a solvent cut asphalt consisting of four parts of 85-100 penetration grade asphalt and five parts of kerosene. The hot elastomeric composition was spread over the tacked area at an average thickness of 0.18 inches and the hot material was completely covered with one fourth inch seal coat aggregate.

At the same time the above patch was applied, a hot mixed sand-asphalt patch was applied to an adjoining area. Four months after application, the elastomeric rubber-asphalt pavement repair patch was still in good condition whereas the sand-asphalt patch was failing. No evidence of spreading or cracking was found in the elastomeric pavement repair patch.

## EXAMPLE IV

The following pavement repair test panels were applied to the same street as described in Example I. An elastomeric composition was prepared from two parts of 85-100 penetration grade asphalt and one part of partially devulcanized reclaimed rubber by weight. The temperature of the asphalt was about 430° F. when the rubber was added and mixed therein. The resulting hot jellied elastomeric composition was spread over an area of two square yards at a rate of one gallon of hot elastomeric material per square yard of pavement area. After application, the hot elastomeric material was completely covered with one-fourth inch seal coat aggregate and turned over to traffic. At the time of application, the atmospheric temperature was 101° F. and the pavement temperature was 138° F. The day after application, the test panel was subjected to nearly an inch of heavy rain. The patch showed no sign of damage although it was subjected to traffic in a completely submerged condition for hours. This patch held up exceedingly well showing no cracking or stripping until it was finally destroyed when the street was rebuilt.

A hot elastomeric composition was prepared from two parts of 85-100 penetration grade asphalt to one part of No. 30 mesh ground whole tire rubber (rubber No. 9306 of U.S. Rubber Reclaiming Co.). The asphalt was heated to a temperature of 450° F. when the rubber was added thereto and mixed therein to form the jellied composition. The hot elastomeric composition was applied to the pavement surface at the rate of 1 gallon of the composition per square yard of street area. After application, the hot elastomeric material was completely covered with one-fourth inch seal coat aggregate and turned over to traffic. At the time of application, the atmospheric temperature of 101° F. and the pavement temperature was 138° F. The consistency of the elastomeric composition was too thick for proper spreading. The resulting patch showed disconnected areas. It appears that the hot elastomeric mixture should consist of relatively greater amounts of 85-100 penetration grade asphalt for best workability when preparing the material from ground whole tire rubber. This patch was also subjected to a heavy rain storm the day after its application. The patch showed no sign of damage although it was subjected to traffic in a completely submerged condition for many hours. Although the surface was rough after application, the surface ironed out under traffic after a period of 1 month. This patch held up in excellent condition without stripping or cracking until it was completely destroyed when the street was rebuilt.

An elastomeric composition was prepared from three parts of 85-100 penetration grade asphalt to one part of No. 30 mesh ground whole tire rubber (Rubber No. 9306 of the U.S. Rubber Reclaiming Co.). The asphalt was heated to a temperature of 400° F. then the rubber was added thereto and mixed therein to form the hot elastomeric composition. The hot elastomeric composition was applied to the street at the rate of one gallon of the composition per square yard of pavement area. After application, the material was completely covered with concrete sand and turned over to traffic. The atmospheric temperature at the time of application was 107° F. officially, the atmospheric temperature three feet above the pavement was 114° F., and the pavement temperature was 156° F. This patch held up exceedingly well until completely destroyed when the street was

rebuilt. At the time of its destruction, it showed no sign of reflection cracking or stripping.

An elastomeric composition was prepared from two parts of 85-100 penetration grade asphalt to one part of No. V-17 Asphalt Soluble Rubber (A product of the U.S. Rubber Reclaiming Co.). The asphalt was heated to a temperature of 410° F. when the rubber was added thereto and mixed therein to form the hot elastomeric composition. The hot elastomeric composition was spread over the pavement area at a rate of one gallon of composition per square yard of pavement surface. After application, the composition was completely covered with concrete sand and turned over to traffic. At the time of application, the atmospheric temperature was 107° F., the atmospheric temperature three feet above the pavement was 114° F. and the pavement temperature was 156° F. This repair patch held exceedingly well until its final destruction when the street was rebuilt. At the time of destruction, the panel showed no sign of reflection cracking or stripping.

As shown in the above examples, a tack coat can be applied before placement of the hot elastomeric material to the pavement surface to be repaired if desired. At first it appeared desirable to have a tack coat for the best results. However, subsequent results show that a tack coat may not be necessary. The important thing is to have the surface of the pavement to be repaired clean of all debris and dry. If the surface is to be tacked, the surface can be tacked with hot asphalt, solvent cut asphalt, emulsified asphalt, or by heating the pavement surface, if it is an asphaltic pavement surface, with a torch to make the surface adhesive and tacky.

#### EXAMPLE V

One hundred grams of 85-100 penetration grade asphalt were weighed into each of four separate beakers. The beakers were labeled No. 1, No. 2, No. 3 and No. 4 and the contents were heated to 350° F., 400° F., 450° F., and 500° F. respectively. Fifty grams of partially devulcanized reclaimed rubber were mixed with the asphalt contents of each beaker to yield the following results:

1. Temperature at time of mixing - 350° F.  
Consistency - thin slurry  
Mixed for 2 min. before observing consistency.  
Consistency after 16 hr. curing at 140° F - soft, sticky, and stringy.  
Consistency after 4 hr. curing at 250° F - soft.
2. Temperature at time of mixing - 400° F.  
Consistency - slurry.  
Mixed for 2 min. before observing consistency.  
Temperature after mixing - 300° F.  
Consistency after 16 hr. curing at 140° F - soft, sticky, and stringy.  
Consistency after 4 hr. curing at 250° F - soft.
3. Temperature at time of mixing - 450° F.  
Temperature after mixing - 330° F.  
Mixed for 2 min. before observing consistency.  
Consistency - thick slurry.  
Consistency after 16 hr. curing at 140° F - semi-soft, not sticky.  
Consistency after 4 hr. curing at 250° F - soft.
4. Temperature at time of mixing - 500° F.  
Temperature after mixing - 350° F.  
Consistency - very thick slurry  
Mixed for 2 min. before observing consistency  
Consistency after 16 hr. curing at 140° F - spongy, not sticky.  
Consistency after 4 hr. curing at 250° F - soft.

The elasticity of the cold elastomeric composition was better with the compositions mixed at the higher temperature and was the best with sample No. 4 which was prepared at 500° F. However, the hot workability of sample No. 4 was very poor at a temperature of 500°

F. Compositions prepared at asphalt temperatures between about 400° and about 450° F. appear to be most satisfactory. The elastomeric composition was somewhat brittle at 19° F. but ductile at 36° F.

#### EXAMPLE VI

The four elastomeric compositions prepared in the previous example were cooled to room temperature. A pea size portion was taken from each sample and placed on a shiny piece of tin plate and the tin plate was placed in the oven at an angle of 30°. The amount of flow for each sample was observed under various temperatures to yield the following results:

|    | [Sample No.]<br>(Mixing Temp.) | [Flow]     |
|----|--------------------------------|------------|
|    | Flow at 170° F for 2 hr.       |            |
| 20 | 1 (350 deg)                    | very small |
|    | 2 (400 deg)                    | none       |
|    | 3 (450 deg)                    | none       |
|    | 4 (500 deg)                    | none       |
|    | Flow at 210° F for 4 hr.       |            |
| 25 | 1 (350 deg)                    | very small |
|    | 2 (400 deg)                    | none       |
|    | 3 (450 deg)                    | none       |
|    | 4 (500 deg)                    | none       |
|    | Flow at 330° F for 2 hr.       |            |
| 30 | 1 (350 deg)                    | 4 in.      |
|    | 2 (400 deg)                    | 2 in.      |
|    | 3 (450 deg)                    | 3 in.      |
|    | 4 (500 deg)                    | none       |

#### EXAMPLE VII

One gallon of the elastomeric pavement repair material made for the last two panels in Example I were molded in a steel concrete cylinder test can. After the mixture had cooled, the cans were removed and the two specimens were removed. Each block measured 6 in. in diameter and 7 to 8 inches in height. The specimen molded from the elastomeric pavement repair material the last patch in Example I was the designated specimen A and the specimen molded from the elastomeric pavement repair material of the next to last patch in Example I was designated as specimen B. These specimens were tested for elasticity (compression and recovery) as follows: The height of each specimen was determined; each specimen was compressed by applying a vertical load until a 2 in. displacement in height was observed. The load was removed in one test immediately, and another test 5 minutes after the 2 in. displacement. The height of each specimen was measured at intervals of 0 time, 1 hour, 12 hours after the load had been removed. The recovery height of each specimen was determined as an indication of the elastic properties of the material. Recovery in inches as the percentage of the 2 in. displacement length, was designated as the percent of the recovery of the elastomeric pavement repair material. The following results were obtained:

#### SPECIMEN A

60 Mixing temperature of asphalt: 440° F.  
Height of test specimen before loading: 7.75 in.  
Height of test specimen with load: 5.75 in.  
Height of test specimen 1 hr. after immediate release of load: 7 in.  
Percent recovery = 1.25/2 = 63 percent.  
Height of test specimen before loading: 6 in.  
Height of test specimen when loaded for 5 min.: 4 in.

Percent recovery (1 hr. after removing load) = 0.5/2  
= 25%.

Height of test specimen 12 hr. after removing load: 5 in.

Percent recovery 12 hr. after removing load = 1 in./2 in. = 50 percent.

#### Consistency Test

Cured for 24 hr. at 140° F.

Observation: sticky and soft.

#### SPECIMEN B

Mixing temperature of asphalt: 420° F.

Height of test specimen before loading: 7 in.

Height of test specimen with load: 5 in.

Height of test specimen 1 hr. after immediate release of load: 6.75 in.

Percent recovery 1 hr. after release of load = 1.75/2 in. = 88 percent.

Height of test specimen when loaded for 5 min: 4.75 in.

Height of test specimen 1 hr. after release of load: 6 in.

Height of test specimen 12 hr. after removing load: 6.50 in.

Percent recovery 1 hr. after removing load applied for 5 min. = 1 in./2 in. = 50 percent.

Percent recovery 12 hr. after removing load applied for 5 min. = 1.5 in./2 in. = 75 percent.

#### Consistency Test

Cured for 24 hr. at 140° F.

Observation: gummy and firm.

It appears that the temperature of the asphalt at the time of mixing with the rubber has an effect on the elastomeric composition product. Specimen B showed more resiliency and elasticity than Specimen A, possibly indicating some damage to the rubber at higher asphalt temperatures. However, in field practice we have found that there is a time-temperature correlation and high asphalt temperatures do not necessarily effect the elastomeric product if the hot composition's high temperature is not maintained for a long period.

The above examples show that the use of either partially devulcanized reclaimed rubber, conventional shredded rubber derived from buffings and reclaimed rubber, ground whole tire rubber, tire buffings, and asphalt soluble rubber together with an asphalt in the proportions of from about 1 part of rubber to about 2 to about 3 parts of asphalt prepared into the elastomeric pavement repair composition of the present invention will prevent reflection cracking from elastic-type failures caused by fatigue cracking of the pavements at a very nominal cost. It is believed that this has never been achieved by skin patching the pavement surfaces with any other material. This should prove to be a boon to maintenance forces throughout the country who are plagued with repairing this type of failure in asphaltic and concrete pavements.

#### EXAMPLE VIII

120-150 penetration grade asphalt was heated to a temperature of 475° F. Rubber tire buffings were added to the hot asphalt in the proportion of three parts of asphalt to one part of rubber. Ninety-eight percent of the rubber passed a No. 25 Sieve (AASHO Designation M-92). The rubber was free from fabric, wire or other contaminating materials. The rubber had a small

amount of calcium carbonate (not more than 4%) which was included to prevent the rubber particles from sticking together. The resulting mixture was mixed for a period of less than 5 minutes to form a jellied semi-fluid material which was the hot elastomeric material. The pavement surface to be repaired was swept clean of all debris and thoroughly dried. The mixture was sprayed onto the pavement surface at a pressure between about 70 and about 100 lbs. per square inch at rate of between 10 1 and 0.75 gallons per square yard of pavement surface area. About 40 lbs. of cover aggregate were spread over the hot elastomeric material after its application. The cover aggregate had a wear percentage of not more than 40 at 500 revolutions as determined by AASHO T-96. The aggregate was clean and free of any coating. Seventy-five percent by weight of the aggregate was retained on a No. 16 Sieve and this portion had at least one fractured face produced by crushing. After the aggregate was spread, it was compacted into the hot elastomeric material with a roller. The application of the aggregate and its compacting was performed within 15 minutes of application of the hot pavement repair material onto the pavement surface.

I have found that when the hot asphalt is heated to a temperature of 440° F. or less, the hot elastomeric pavement repair material prepared therefrom requires more than 5 minutes of mixing with the rubber. In such a situation, preferably 95% of the rubber shall pass a No. 16 Sieve and not more than 15% of the rubber shall pass 25 a No. 25 Sieve. When the asphalt is heated to a temperature between 440° and 500° F., the hot elastomeric material is formed in less than five minutes after the rubber has been added and mixed with the hot asphalt. At the temperatures of 475° and 500° F., the hot elastomeric composition is frequently formed in a matter of seconds. When the composition is prepared with asphalt at temperatures in excess of 440° F., preferably 98% of the rubber shall pass a No. 25 Sieve.

In geographical areas where the temperatures seldom go below freezing, an excellent elastomeric pavement repair material can be prepared from about three parts asphalt to about one part rubber. In areas where freezing occurs more than once or twice during the year an excellent elastomeric pavement repair material can be prepared from about 7 parts asphalt and about 3 parts rubber by weight.

When a large surface is to be repaired, and several panels are to be laid, all joint edges of the previous laid patches should be swept clean of overlapping cover material. Naturally precaution should be taken to avoid skips and overlaps at joints to protect the surfaces of adjacent structures from being spattered or marred when opened to vehicular traffic.

After application of the present elastomeric pavement repair material and aggregate, the surface of the street is only raised approximately three-eighths of an inch in height so it does not significantly reduce curb height or interfere with or require changes in subsurface drainage construction, manhole covers and the like.

The present elastomeric pavement repair composition ages far more slowly than conventional asphalt pavement compositions. A combination of the rubber and asphalt as set forth in this application seem to mutually protect against oxidation and degradation. The composition remains pliable and elastic over a period of many years.

The elastomeric pavement repair material of the present invention has been employed in many pavement

services with very satisfying results. The material has been applied to U.S. Highway 66 near Williams, Ariz. This highway is subject to heavy vehicular traffic and also to wide variations in weather. During the summer, the highway is blistering hot and during the winter, the highway is subject to subzero temperatures. However, the portion of the highway repaired with the elastomeric composition has withstood these conditions for over five years without any crack reflection or other deleterious affects. In addition, this material has been used to repair airport runways, taxiways, refueling areas and access roads. Runway areas repaired with this material have been able to withstand the repeated pounding of large jet airliners such as the Boing 747, which weigh more than 500,000 lbs. without damage to the repair patch. It has been demonstrated and proven that the present elastomeric pavement repair material will outlast conventional patching materials many times over.

The elastomeric pavement repair composition of the present invention has much lower temperature susceptibility than conventional asphalt and is less prone to brittleness in cold weather and bleeding in hot weather.

The adhesion characteristics of the elastomeric pavement repair material in the presence of water have proven to be far superior to that of asphalt alone and the susceptibility of aggregate stripping has been reduced to a level far below that of normal asphalt-aggregate pavement.

When the hot elastomeric pavement repair material is applied as a membrane over a pavement area, it forms an impervious surface or layer which prevents the entry of water through the cracks to enter the base and subgrade underlying the pavement surface. This results in a long term stabilization of the subgrade and base moisture which tends to reduce the magnitude of the deflections in the more stabilized subgrade. The rapid progression of local failure is often due to reduced subgrade support caused by the entrance of surface water through the surface cracks in the pavement.

Small localized areas which require repair may be repaired with the hot elastomeric pavement repair composition by using a conventional concrete pavement rubberized asphalt joint filling kettle, oil jacketed type for mixing and spreading the material. This type of equipment has a self-contained agitator and positive displacement pump for mixing and applying the hot elastomeric pavement repair composition. The composition can be placed on small areas using a spray nozzle or using a joint filling wand. The material may be spread and smoothed with a squeegee. The material can then be dressed by hand sanding or covering with aggregate chips.

#### EXAMPLE IX

An hot elastomeric material prepared from 120-150 penetration grade asphalt which was heated to a temperature between about 350° and 400° F. Ground tire rubber, 16-25 mesh was added to the hot asphalt in the proportions of 3 parts of asphalt to about 1 part rubber. The resulting mixture was stirred causing the mixture to become a jellied composition which occurred within one-half to 1 hour after the introduction of the rubber. The addition of the rubber cooled the resulting mixture by about 50° F. The hot elastomeric material was then sprayed onto the pavement area to be repaired which has been first brushed clean of all foreign debris and

dressed with aggregate. After the material had cooled, the loose aggregate was swept off the surface.

The elastomeric composition can be used to completely surface old and new pavements or roofs. It can be used to form a waterproof membrane for a road base or a waterproof liner for canals, reservoirs, ponds, including leaching and solar ponds, tanks, culverts and pipes. The composition can also be used as an underseal, sound deadening material, joint and crack filler, binder or as a membrane material to combat soil erosion.

#### EXAMPLE X

A main taxiway pavement of a large airport was in very bad condition with extensive alligator cracking together with a number of depressions where settlement had taken place. When it rained, the rain did not lie in these depressions, but rather promptly drained through the cracks into the sub-base creating further distress. This runway was repaired with the elastomeric repair composition by the above described method. Thereafter, the depressions held rainwater until the rainwater completely evaporated. A year after the application, it was decided to place a conventional leveling course of fine, dense graded asphalt concrete over this surface to smooth out the depressions. This leveling, of course, varied in thickness from a fraction of an inch to approximately 4 inches. After being in service approximately 2 years, it was noted that the leveling course had begun to show reflection cracking and some subsidence due to differential compaction in the thicker areas. However, it was noted that water did not penetrate into the base as it had done in the original surface indicating that the underlying elastomeric pavement repair membrane was still intact. This membrane did not stop vertical movement; accordingly, the relatively brittle leveling course was subject to fatigue cracking while the underlying elastomeric membrane was elastic enough to take the vertical movement without cracking.

#### EXAMPLE XI

85-100 penetration grade asphalt was heated to a temperature about 420° F and then mixed with ground partially devulcanized reclaimed rubber. The portions of asphalt and rubber were two to one by weight. The rubber was mixed with hot asphalt until a thick jellied composition formed which had the viscosity of a thick pancake batter. The hot elastomeric material was applied to a clean pavement surface at the rate of a half gallon of hot material per square yard of pavement area. The hot elastomeric material was completely covered after application with one-half inch seal coat aggregate. Four years after this patch was applied, the patch was still in excellent condition with no stripping or cracking observed.

An adjacent patch was made with the same above material at the same time except the composition was applied at a rate of one gallon hot material per square yard of pavement area. After four years of use, the patch was still in excellent condition showing no reflection cracks, surface wear or shoving of the material.

#### EXAMPLE XII

60-70 penetration grade paving asphalt was heated to a temperature of about 390° F. Ground tire rubber (particle size 0.044 inch) was added to the hot asphalt and thoroughly mixed therein for 10 minutes while heating was continued to form a hot thick jellied mixture. The

rubber and asphalt were added in the portions of one part rubber to two parts asphalt.

Other penetration grade asphalts such as 10 through 300 penetration grades can be used in preparation of the hot elastomeric material; for example, 10-10, 10-20, 40-50, 70-80, 85-100, 120-150 and 200-300 penetration grade asphalts can also be employed.

### EXAMPLE XIII

Paving grade asphalt, 85-100 penetration grade, was heated to about 425° F. Granular scrap rubber was added to the hot asphalt in the weight ratios of about 75% asphalt to about 25% rubber and mixed. The resulting mixture was mixed until a hot viscous gel composition was formed. The hot viscous gel composition was applied to a paper backing having a release type surface. The composition was poured into a form and screed to form a layer having an average thickness of about one-eighth inch. About a half gallon of the composition was applied per square yard of backing. Immediately thereafter, a half gallon of light-weight aggregate was applied to the surface of the hot elastomeric material and rolled therein. After the hot elastomeric material had cooled to form the elastomeric cold patch, the surface of the patch was brushed off to remove all loose aggregate. The form was removed and the finished elastomeric cold patch was dusted with hydrated lime as an adhesive breaker.

### EXAMPLE XIV

The first hot jellied elastomeric composition prepared in Example I is applied to a sheet of newspaper as a thin layer. About 1 gallon of the hot composition is applied to each square yard of newspaper. Immediately after application of the hot composition, 40 pounds of nominal three-eighth inch mineral aggregate is applied to the exposed surface of the hot composition and worked therein. An elastomeric cold patch is obtained after the hot composition has cooled.

Similar cold patches can be made from the other hot jellied elastomeric compositions of Examples I-IX, XI and XII inclusive.

Repair of the pavement subject to cracking is accomplished by sweeping the area to be repaired free of all debris and drying it. The pavement surface is tacked with solvent cut asphalt. The elastomeric cold patch is applied to the tacked area and rolled thereon to insure good adhesion between the cold patch and the surface of the pavement. The paper side of the cold patch faces upward.

The pavement surface can be tacked with conventional tacking composition such as asphalt and rubberized bitumen. If the pavement surface is asphaltic, the surface can also be tacked by heating the surface with a torch or by applying asphalt solvent.

### EXAMPLE XV

The hot jellied elastomeric composition of Example V was applied to a flexible sheet and formed into a layer. The sheet had a release type backing prepared from polyvinyl chloride. The hot composition was applied to the release type backing. About 0.4 pounds of the hot composition were applied per square yard of sheet. While the composition was still hot, 20 pounds of nominal three-eighths inch mineral aggregate were applied to the hot composition and worked therein. After the hot composition had cooled, an elastomeric cold patch was obtained.

The pavement is repaired by cleaning the area to be repaired of all debris and dried. The area is tacked with asphalt. The elastomeric cold patch is cut to size so that its edges extend 6 inches beyond on all sides of the area to be repaired. The sheet is removed from the elastomeric cold patch and the cold patch is applied raw side down to the tacked area. The raw side, is the side which was attached to the sheet. The elastomeric cold patch is tamped and rolled to insure good adhesion between the pavement surface and the cold patch.

### EXAMPLE XVI

The hot jellied elastomeric composition of Example VII is mixed with an equal amount by weight of nominal one-fourth inch aggregate. The resulting mixture is applied to a polyethylene film. About one-half gallon of the composition is applied per square yard of the polyethylene sheet. The exposed surface of the mixture is dressed with sand. After the hot composition cools, the resulting elastomeric cold patch is dusted with lime.

An asphaltic pavement to be repaired is swept clean of all debris and dried. The area to be repaired is tacked with kerosene. The elastomeric cold patch is applied to the tacked area with the polyethylene sheet facing upwards. The cold patch is tamped and rolled on to the pavement to insure good adhesion between the patch and the pavement surface.

### EXAMPLE XVII

85-100 penetration grade asphalt was heated to a temperature of about 420° F. and then mixed with ground partially devulcanized reclaimed rubber. The portions of asphalt and rubber were two to one by weight. The rubber was mixed with hot asphalt until a thick jellied composition formed which had the viscosity of a thick pancake batter. The hot elastomeric material was applied to a clean pavement surface at the rate of a half gallon of hot material per square yard of pavement area. The hot elastomeric material was completely covered after application with one-half inch seal coat aggregate. Four years after this patch was applied, the patch was still in excellent condition with no stripping or cracking observed.

An adjacent patch was made with the same above material at the same time except the composition was applied at a rate of one gallon hot material per square yard of pavement area. After four years of use, the patch was still in excellent condition showing no reflection cracks, surface wear or shoving of the material.

### EXAMPLE XVIII

The following panels were prepared according to the procedure of Example XXI.

Panel No. 3 was prepared from "Golden Bear" 85-100 penetration grade asphalt, 16-24 mesh rubber buffings supplied by Atlos Rubber Company of Los Angeles, California (hereinafter referred to as "Atlos rubber") and minus three-eighths aggregate chips. One part rubber was mixed with two parts of asphalt by weight at 425° F. The chips were preheated (450° F.) and spread on heavy paper backing; the asphalt-rubber mixture was poured over the chips to form an elastomeric cold patch.

Panel No. 4 was prepared from "Santa Maria" 85-100 penetration grade asphalt, Atlos rubber (16-24 mesh) and —three-eighths inch aggregate chips in the same manner as panel No. 3.

Panel No. 5 was prepared from Edington 85-100 penetration grade asphalt, Altos rubber (-24 mesh) and -three-eighths inch chips. One part rubber was mixed with three parts asphalt by weight at 425° F. Hot aggregate chips (450° F.) were added to the resulting hot elastomeric composition in an equal weight portion, that is an amount of chips equal in weight and amount of the hot elastomeric composition, and mixed. The resulting mixture was spread on thin paper backing to form an elastomeric cold patch having an area of approximately 4 square feet and a thickness of about one-fourth inch.

Panel No. 6 was prepared from Edington 85-100 penetration grade asphalt, Altos rubber (16-24 mesh) and -three-eighths inch chips. One part rubber was mixed with two parts asphalt by weight at 425° F. The resulting hot elastomeric mixture was spread on release paper and the exposed surface of the hot composition was coated with pre-heated chips (450° F.).

What is claimed is:

1. The method of repairing pavement subject to 20 cracking which comprises the steps of:

preparing a hot elastomeric pavement repair material consisting essentially of paving grade asphalt and hydrocarbon rubber by mixing the paving grade asphalt and the hydrocarbon rubber in a ratio of 25 about one to about three parts asphalt to about one part rubber at a temperature within the range of about 300 and about 500° F. to form a jellied composition, the mesh size of the rubber being from about -16 to +200;

treating the surface of the pavement area to be repaired with adhesive means to make the surface tacky and adhesive;

applying a layer of the hot elastomeric material over 30 the pavement to be repaired at a rate of about 0.3 to about 1 gallon of hot elastomeric material per square yard of repaired pavement area;

applying a dressing of aggregate cover having a nominal size of about one-fourth to about three-eighths inches over the top surface of the hot elastomeric material layer; and

working the aggregate into the hot elastomeric material, the aggregate being applied at a rate of about 25 to about 40 pounds of aggregate per square yard of the hot elastomeric material layer.

2. The method according to claim 1 wherein the hydrocarbon rubber is selected from the group consisting of ground whole tire rubber, reclaimed rubber, partially devulcanized reclaimed rubber, asphalt soluble reclaimed rubber, rubber buffings, ground tire tread rubber, and ground innertube rubber

3. The method according to claim 1 wherein the paving grade asphalt is 85-100 penetration grade asphalt.

4. The method according to claim 1 wherein the paving grade asphalt is 120-150 penetration grade asphalt.

5. The method according to claim 1 wherein the hot jellied composition is prepared from about two to about three parts of asphalt to about one part rubber.

6. A method of making a road which comprises the steps of:

grading an area wherein a road is to be located to form a subgrade of the road;

compacting the top portion of the subgrade to form a 65 base layer;

preparing a hot elastomeric pavement material by mixing paving grade asphalt and hydrocarbon rub-

ber in the ratio of about one to about three parts asphalt to about one part rubber at a temperature from about 350° F. to about 500° F. to form a hot jellied composition; and

applying the hot elastomeric material over the base layer at a rate of about  $\frac{1}{4}$  to about 2.5 gallons of hot elastomeric material per square yard of base layer.

7. The method according to claim 6 wherein an aggregate dressing is applied to the surface of the applied hot elastomeric material before the material sets up at the rate of about 20 pounds to about 50 pounds of aggregate per square yard of applied hot material; and working the aggregate into the hot material.

8. The method according to claim 6 wherein the compacted base layer is treated with a binder, cement, asphalt or cutback asphalt prior to applying the hot elastomeric material.

9. The method according to claim 6 wherein a drainage ditch is excavated along one side of the subgrade prior to applying the hot elastomeric material, and the hot elastomeric material is applied on the bottom and back slopes of the drainage ditch at a rate of about  $\frac{1}{4}$  to about 2.5 gallons of hot elastomeric material per square yard of drainage ditch surface.

10. The method according to claim 9 wherein the hot elastomeric material is applied to the outer top edge and shoulder of the drainage ditch.

11. The method according to claim 10 wherein an aggregate dressing is applied to the hot elastomeric material before the composition sets up, at a rate of between about 20 to about 50 pounds of aggregate per square yard of applied material, and the aggregate dressing is worked in the hot material.

12. The method according to claim 6 wherein two drainage ditches are excavated along the sides of the subgrade prior to applying the hot elastomeric material, and the hot elastomeric material is applied on the bottom and back slopes of the drainage ditches at a rate of about  $\frac{1}{4}$  to about 2.5 gallons of hot elastomeric material per square yard of drainage ditch surface.

13. The method according to claim 12 wherein the hot elastomeric material is applied to the outer top edge and shoulders of the two drainage ditches.

14. The method according to claim 13 wherein an aggregate dressing is applied to the hot elastomeric material before the composition sets up, at a rate of between about 20 to about 50 pounds of aggregate per square yard of applied material, and the aggregate dressing is worked into the hot material.

15. The method according to claim 6 where an intermediate layer of asphalt, asphalt-concrete, or concrete is constructed over the base layer and the hot elastomeric material is applied to the intermediate layer.

16. The method according to claim 6 wherein the subgrade is compacted with gravel, sand and aggregate to form a base layer prior to applying the hot elastomeric material.

17. The method according to claim 16 wherein the base layer is treated with a binder, cement, asphalt or cutback asphalt prior to applying the hot elastomeric material.

18. A method of making a road which comprises the steps of:

(a) grading an area wherein a road is to be located to form a subgrade of the road;

(b) compacting the subgrade with gravel, sand or aggregate to form a base layer;

- (c) excavating a drainage ditch along one side of the subgrade;
- (d) preparing a hot elastomeric repair material by mixing paving grade asphalt and hydrocarbon rubber in the ratio of about one to about three parts asphalt to about one part rubber at a temperature of from about 350° F. to about 500° F. to form a hot jellied composition;
- (e) applying the hot elastomeric material over the base layer and the drainage ditch at a rate of about  $\frac{1}{4}$  to about 2.5 gallons of hot elastomeric material per square yard of base layer and drainage ditch;
- (f) applying an aggregate dressing to the surface of the hot elastomeric material before the material sets up at the rate of about 20 pounds to about 50 pounds of aggregate per square yard of applied hot material; and
- (g) working the aggregate in the hot material.

19. The method according to claim 18 wherein the compacted base layer is treated with a binder, cement, asphalt or cutback asphalt prior to applying the hot 20 elastomeric material.

20. The method according to claim 18 where the hot elastomeric material is applied to the out top edge and shoulder of the drainage ditch, an aggregate dressing is applied to the hot elastomeric material before the material sets up at a rate of between about 20 to about 50 pounds of aggregate per square yard of applied material, and the aggregate dressing is worked into the hot material.

21. The method according to claim 18 where an intermediate layer of asphalt, asphalt-concrete, or concrete is constructed over the base layer and the hot elastomeric material is applied to the intermediate layer.

22. The method according to claim 18 wherein the hydrocarbon rubber is selected from the group consisting of ground whole tire rubber, reclaimed rubber, partially devulcanized reclaimed rubber, asphalt soluble rubber, reclaimed rubber, rubber buffings, ground tire tread rubber and ground innertube rubber; and the asphalt is selected from the group consisting of 10-10, 40-50, 60-70, 70-80, 85-100, 120-150, and 200-300 40 penetration grade asphalt.

23. The method according to claim 18 wherein the paving grade asphalt is 85-100 penetration grade asphalt.

24. The method according to claim 18 wherein the paving grade asphalt is 120-150 penetration grade asphalt.

25. The method according to claim 18 wherein the sized aggregate has a nominal size of from about  $\frac{1}{4}$  to about three-eighths inches.

26. The method of treating pavement subject to cracking which comprises the steps of:

- preparing a hot elastomeric pavement repair material by mixing paving grade asphalt and hydrocarbon rubber in a ratio of about one to about three parts asphalt to about one part rubber at a temperature within the range of about 300 and about 500° F. to form a jellied composition, the mesh size of the rubber being from about -16 to +200;
- treating the surface of the pavement area to be repaired with adhesive means to make the surface tacky and adhesive; applying a layer of the hot elastomeric material over the pavement to be repaired to form a stress absorbing interlayer membrane having a thickness of about 0.1 to about 0.5 inch; and applying a pavement layer of pavement surfacing materials selected from the group consisting of asphalt-concrete, macadam and concrete over the interlayer membrane.

27. The method according to claim 26 where a dressing of aggregate cover having a nominal size of about one-fourth to about three-eighths inches is applied over the top surface of the interlayer membrane prior to applying the pavement layer and the aggregate is worked into the hot elastomeric material, the aggregate being applied at the rate of about 25 to about 40 pounds of aggregate per square yard of the hot jellied composition layer.

28. A method of treating pavement subject to cracking which comprises the steps of:

preparing a hot elastomeric pavement repair material by mixing paving grade asphalt and hydrocarbon rubber in a ratio of about one to about three parts asphalt to about one part rubber at a temperature within the range of about 300° and about 500° F. to form a jellied composition, the mesh size of the rubber being from about -16 to +200;

applying a layer of the hot elastomeric material over the pavement to be repaired to form a stress absorbing interlayer membrane having a thickness of about 0.1 to about 0.5 inch; and applying a pavement layer of pavement surfacing materials selected from the group consisting of asphalt-concrete, macadam and concrete over the interlayer membrane.

29. The method according to claim 28 where a dressing of aggregate cover having a nominal size of about one-fourth to about three-eighths inches is applied over the top surface of the interlayer membrane prior to applying the pavement layer and the aggregate is worked into the hot elastomeric material, the aggregate being applied at the rate of about 25 to about 40 pounds of aggregate per square yard of the hot jellied composition layer.

30. A method of repairing pavements which includes the steps of:

treating the area of the pavement surface to be repaired with adhesive means to make the area adhesive and tacky; and

securing an elastomeric cold patch on the treated area, said elastomeric cold patch comprising a layer of aggregate and an elastomeric pavement repair material and a thin flexible sheet attached to one side of the layer, the elastomeric material consisting essentially of 10 through 300 penetration grade asphalt and hydrocarbon rubber which have been mixed together in the ratio of from about one to about three parts asphalt to about one part rubber by weight at a temperature from about 300 to about 500° F. to form a hot jellied composition, the cold patch being applied to the treated pavement with the thin flexible sheet side up.

31. The method of repairing pavements which includes the steps of:

treating the area of the pavement surface to be repaired with adhesive means to make the area adhesive and tacky; and

securing an elastomeric cold patch on the treated area, said elastomeric cold patch comprising a layer of aggregate and an elastomeric pavement repair material and a thin flexible sheet attached to one side of the layer, the elastomeric material consisting essentially of 10 through 300 penetration grade asphalt and hydrocarbon rubber which have been mixed together in the ratio of from about one to about three parts asphalt to about one part rubber by weight at a temperature from about 300 to about 500° F. to form a hot jellied composition, the cold patch being applied to the treated pavement with the thin flexible sheet side down.

\* \* \* \* \*